

Aug. 4, 1953

J. H. PFAU

2,647,285

## METHOD FOR CRIMPING TEXTILE FIBERS

Filed July 20, 1950

2 Sheets-Sheet 1



Fig. 1.



Fig. 2.

Fig. 3.



Fig. 4.

JULIUS H. PFAU INVENTOR

BY   
ATTORNEY

Aug. 4, 1953

J. H. PFAU

2,647,285

METHOD FOR CRIMPING TEXTILE FIBERS

Filed July 20, 1950

2 Sheets-Sheet 2



JULIUS H. PFAU

BY

*Offeek*  
ATTORNEY

## UNITED STATES PATENT OFFICE

2,647,285

## METHOD FOR CRIMPING TEXTILE FIBERS

Julius H. Pfau, Yonkers, N. Y., assignor to Alexander Smith, Incorporated, a corporation of New York

Application July 20, 1950, Serial No. 174,870

5 Claims. (Cl. 19—66)

1

This invention relates to a method and apparatus for improving the characteristics of textile fibers and more particularly for imparting a controlled artificial crimp to such fibers.

An object of the invention is to provide a novel and improved method and apparatus for the above purpose.

Another object is to provide an apparatus for crimping and setting textile fibers in which the crimping and setting operations may be controlled independently.

Various other objects and advantages will be apparent as the nature of the invention is more fully disclosed.

The invention is particularly applicable to animal fibers of short fiber lengths such as wool. It may also be applied, however, to other fibers, including vegetable fibers such as cotton, jute, hemp, ramie and flax, continuous filaments such as silk or uncrosslinked thermoplastic synthetic fibers such as rayon, nylon, or the like, depending upon the conditions maintained in the crimping and setting zones.

In accordance with the present invention the fibers are crimped mechanically and the crimp is set into the fibers in a separate setting zone. The mechanical crimp may be imparted in various ways as by feeding a rope or slubbing of fibers between feed rolls into a mass of fibers held under a back pressure sufficient to cause the fibers to be folded over and crimped as they are forced into the mass. In a further embodiment the fibers are crimped in a gear crimper comprising a pair of fluted rolls, either cylindrical or conical, between which the fibers are passed, or by means of a pair of belts having serrated surfaces and held together under sufficient pressure to cause the fibers to be distorted and crimped as they pass therebetween. If the nature of the fibers so requires they may be pre-treated to soften the same sufficiently to permit the crimping.

The fibers thus treated have a crimp which is temporary and unset. In order to set the crimp thus formed the fibers are introduced into a zone wherein a mass of fibers are compacted and held under pressure and are treated with a setting agent while the compacting pressure is maintained. The setting agent may be introduced into the mass of fibers in a stuffing box wherein they are held under pressure, or the fibers may be compacted and packaged or baled under pressure and introduced into a setting chamber containing a setting agent, such as steam under pressure or a heated liquid, such as a dye bath. In

2

either case the fibers are held under pressure and the treatment is carried out for a time to effect a permanent set which remains in the fibers after they have been released from the compacting force.

The novel features which are characteristic of this invention will be better understood by referring to the following description, taken in connection with the accompanying drawings in which specific embodiments have been set forth for purposes of illustration.

In the drawings:

Fig. 1 is a sectional view illustrating a crimper and stuffing box embodying the present invention;

Fig. 2 is a sectional view illustrating a setting apparatus in which the fibers are held in compacted form in a dye bath;

Fig. 3 is a similar sectional view illustrating the setting step as carried out in a steam chamber;

Fig. 4 is a sectional view illustrating a further embodiment of the invention wherein the fibers are set while held compacted in a setting chamber;

Fig. 5 is a sectional view illustrating an embodiment of the invention wherein the fibers are crimped by gear crimpers and are set in a stuffing box;

Fig. 6 is a sectional view illustrating the invention as applied to a pair of belts having serrated crimping surfaces;

Fig. 7 is an enlarged sectional view illustrating a cone crimper; and

Fig. 8 is a section taken on the line 8—8 of Fig. 7.

Referring to the drawings more in detail, the invention is shown in Fig. 1 as applied to a stuffer crimper comprising a pair of feed rolls 10 which are driven in any suitable manner and between which a rope or slubbing 11 is passed for crimping. A pivoted gate 12 mounted on a pedestal 13 by means of a pivot 14 and provided with a counterweight 15 is formed with a surface 16 which is adapted to engage the surfaces of the feed rolls 10 and to form in combination with said feed rolls 10 a closed crimping chamber 17 containing a mass of fibers which are held compacted under a pressure determined by the position of the counterweight 15. The surface 16 is shown as sloping to the left to provide an inclined path over which the fibers, after being crimped in the chamber 17, are discharged as a rope 20 of crimped fibers. The crimped fibers are thus discharged from the chamber 17 when

the pressure built up in the chamber 17 is sufficient to overcome the weight 15 and cause the gate 12 to pivot about its pivot 14.

In order to build up this pressure the incoming fibers are fed by the feed rolls 10 into the mass of fibers already in the crimping chamber 17 and are folded over to form spaced crimps as they are introduced against the compacted mass of fibers already in the chamber. Hence the rope 20 emerging from the chamber 17 is composed of fibers having a series of crimps the frequency of which is dependent upon the nature of the fibers and the pressure exerted upon the gate 12 by the weight 15.

In the embodiment shown in Fig. 1 the rope 20 is introduced through a hopper 21 into a standard baler shown as a cylinder 22 having an end closure 23 which is secured to the cylinder walls by suitable means such as a hinge 24 and a latch 25, and having a piston 26 for compacting the mass of fibers in the cylinder. As the rope 20 is fed into the cylinder 22 the piston 26 may be reciprocated for packing the mass of fibers against the end closure 23 and when the cylinder 22 has been filled the piston 26 is advanced under suitable pressure to compact and compress the fibers against the end wall 23 in a compact mass 27. The mass of fibers 27, while still held under pressure by the piston 26, is then baled by suitable means, as by wires 29 which may be inserted in the cylinder in the usual manner to form a bale 28 secured and held under a substantial compacting pressure by wires 29. The bale of fibers 28 may be removed from the cylinder 22 by releasing the latch 25 and may be introduced into a setting zone or may be stored for future setting.

Fig. 2 illustrates one method of setting the crimp in the baled fibers wherein a plurality of bales 28, mounted on a movable platform 30 are positioned in a tank 31 which may contain a setting agent such as a solution 32 which is circulated through the bales by means of a circulating impeller 33. Suitable steam pipes 34 are provided for maintaining the solution at a proper temperature. The solution may include a dye in which case the setting is combined with the dyeing step. The bales are shown as extending substantially entirely across the tank so that the liquid must pass therethrough as it is recirculated by the impeller.

The fibers are maintained in the bath for a sufficient period of time to effect a permanent set of the crimp, after which they may be removed and the pressure thereon released as by removing the wires 29. The fibers may then be carded and spun or otherwise treated in the usual manner.

In the embodiment shown in Fig. 3 the bales 28 are shown as placed in a steam chamber 40 wherein steam is introduced through a pipe 41 and is maintained under suitable conditions of temperature and pressure to effect the setting of the crimp. The chamber is vented by pipe 42. After the crimp has been set the bales 28 are removed from the steam chamber and carded and spun in the usual manner. As in Fig. 2, the bales extend entirely across the steam chamber so that the steam must pass therethrough in its path from the inlet pipe 41 to the discharge pipe 42.

Referring to Fig. 4, the crimped rope 20, as received from the crimper of Fig. 1 for example, is introduced by means of a pivoted guide 42 to one of two cylinders 43, each of which is pro-

vided with a piston 44 for compacting the fibers therein and with a hinged gate 45 at the bottom for releasing the fibers after treatment. The gates 45 are secured to the cylinders 43 by means of hinges 46 and may be latched by latches 47. A manifold 48 extends around each of the cylinders 43 and is provided with a plurality of ports 49 for introducing a setting agent into the cylinder. The setting agent, such as steam, is introduced to the manifold 48 by means of an inlet pipe 50. The set fibers may be discharged from the cylinders 43 onto a moving conveyor 51.

In the operation of this device the fibers are introduced into one of the cylinders 43 (the right cylinder as indicated in Fig. 4) by means of the guide 42. After the right cylinder 43 has been filled to the desired level the guide is shifted to the dotted position shown in Fig. 4 to introduce the fibers into the left cylinder, whereupon the piston 44 of the right cylinder is depressed for compacting the fibers in that cylinder against the gate 45. While the mass of fibers is thus held compacted the setting agent, such as steam or superheated water, is introduced through the pipe 50, manifold 48, and ports 49 into the compacted mass of fibers in the cylinder under conditions to set the crimp therein. After a predetermined time the gate 45 is released and the fibers are removed from the cylinder 43 onto the conveyor 51. The gate 45 is then closed and the piston 44 elevated to receive a new supply of fibers. The operation is repeated in the left cylinder.

This apparatus permits the fibers to be received continuously from the crimper and to be set in batches as desired. Obviously the rope 20 from a plurality of crimpers may be fed into the cylinders 43 as above indicated and the entire mass of fibers from all of the crimpers may be set at intervals depending upon the capacity of the cylinders 43.

Referring to the embodiment of Fig. 5 a gear crimper is shown as comprising a pair of fluter rolls 55 which receive a slubbing 11 of fibers to be crimped and discharge the crimped fibers into a hopper 56 of a continuous crimper comprising a cylinder 57 having an end closure 58 and having a reciprocating piston 59. The end closure 58 is shown as hinged by a hinge 60 and is held closed by a compression spring 61. The piston 59 is adapted to be oscillated so as to pack the fibers in the cylinder 57 as they are received from the hopper, to maintain the fibers under substantial pressure therein and to force the fibers out of the cylinder 57 when sufficient pressure is exerted to overcome the force of the spring 61 and open the gate 58. The cylinder 57 is provided with a pair of manifolds 63 having ports 64 communicating with the interior of the cylinder 57 and supplied with an inert medium such as air under pressure through pipes 65, so as to provide an air lock to prevent the escape of the setting agent. The cylinder 57 is also provided with a plurality of manifolds 66 having ports 67 communicating with the cylinder 57 through which a setting agent, such as steam or superheated water, is introduced as by means of pipes 68.

In the operation of this embodiment of the invention the crimped fibers from the gear crimper 55 are held under pressure in the setting chamber 57 during such period as may be required to effect setting of the crimp due to the action of the steam or other setting agent which is introduced through the pipe 68.

The embodiment of Fig. 6 is similar to that of Fig. 5 with the exception of the crimper. In Fig. 6 a pair of conveyor belts 18 are provided having raised members 71 thereon forming a fluted or serrated surface, the members 71 of the two belts being interleaved whereby the rope 11 will be serrated or crimped as it is fed between the belts and conveyed thereby to a discharge point where it is discharged as a crimped rope 20 into the hopper 56 of a crimping chamber 57 as above described.

In the embodiment of Figs. 7 and 8 the crimping of the slubbing 11 is effected by a fluted cone 75 bearing against the surface of a smooth faced cone 78. The slubbing 11 passes around the fluted cone 75 and advances toward the apex thereof. During this passage the fibers are forced into the corrugations of the cone 75 and are crimped, the crimped fibers being discharged as a rope 28 to the hopper 56 as above described.

It is to be understood that the various crimpers of Figs. 1, 5, 6 and 7 may be used in combination with any of the setting devices of Figs. 2, 3, 4 and 5 and that selected combinations have been shown for purposes of illustration only.

In the above method, the raw fibers are first opened, scoured, washed and dried in the usual manner to form stock and under the desired conditions to leave the stock with the desired pH for crimping. The stock is then carded and formed into a condensed rope or slubbing which is fed to the crimpers above described where it is crimped. It is then compacted and set in any of the various setting zones illustrated. For equilibrium conditions of moisture content and pH the setting time varies inversely with the temperature. With steam at a pressure of 20 pounds per square inch the setting time may constitute a few minutes, whereas with hot water or hot dye bath, a setting time of several hours may be required. In any event the mass of fibers is held under compacting pressure during the setting step.

What is claimed is:

1. The method of imparting a permanent artificial crimp to textile fibers, which comprises gripping said fibers between closely spaced conveyor surfaces discharging into a substantially closed zone, and forcing the gripped fibers into said zone against the pressure of a mass of fibers held compacted under pressure in said zone, said pressure being adapted to cause the fibers to be progressively folded over and crimped as they are delivered from said conveyor surfaces, removing the crimped fibers from said zone and releasing the compacting pressure thereon, transferring the fibers while free from said compacting pressure to a second pressure zone, applying

pressure in said last zone to compress said fibers into a compacted mass, and subjecting said mass while under said compacting pressure to a setting agent for a period of time to effect a permanent set of said crimp.

2. The method of imparting a permanent artificial crimp to textile fibers, which comprises gripping said fibers between closely spaced conveyor surfaces discharging into a substantially closed zone, and forcing the gripped fibers into said zone against the pressure of a mass of fibers held compacted under pressure in said zone, said pressure being adapted to cause the fibers to be progressively folded over and crimped as they are delivered from said conveyor surfaces, removing the crimped fibers from said zone and releasing the compacting pressure thereon, transferring the fibers while free from said compacting pressure to a second pressure zone, applying pressure in said last zone to compress said fibers into a compacted mass, introducing a setting agent into said compacted mass of fibers, and maintaining said compacting pressure on said mass until the crimp has been permanently set therein.

3. The method of imparting a permanent artificial crimp to textile fibers, which comprises gripping said fibers between closely spaced conveyor surfaces discharging into a substantially closed zone, and forcing the gripped fibers into said zone against the pressure of a mass of fibers held compacted under pressure in said zone, said pressure being adapted to cause the fibers to be progressively folded over and crimped as they are delivered from said conveyor surfaces, removing the crimped fibers from said zone and releasing the compacting pressure thereon, transferring the fibers while free from said compacting pressure to a second pressure zone, applying pressure in said last zone to compress said fibers into a compacted mass, introducing said compacted mass of fibers into a setting zone, and treating the mass in said setting zone while maintaining said compacting pressure thereon with a setting agent under conditions to effect a permanent set of said crimp.

4. The method set forth in claim 1 in which said setting agent comprises a heated fluid.

5. The method set forth in claim 1 in which said setting agent comprises steam.

JULIUS H. PFAU.

References Cited in the file of this patent

UNITED STATES PATENTS

| 55 | Number    | Name     | Date          |
|----|-----------|----------|---------------|
|    | 332,514   | Hamilton | Dec. 15, 1885 |
|    | 2,311,174 | Hitt     | Feb. 16, 1943 |